

Nov. 30, 1954

A. A. SMITH, JR., ET AL

2,695,845

ANTIMONIAL LEAD ALLOYS

Filed Feb. 15, 1950

Fig. 1



15% Sb, 10% Sn, S nil, bal. Pb. Magnification 100 X — Etchant, Acetic Acid + H<sub>2</sub>O<sub>2</sub>.

Fig. 1a



15% Sb, 10% Sn, 0.0025% S, bal. Pb. Magnification 100 X — Etchant, Acetic Acid + H<sub>2</sub>O<sub>2</sub>.

Fig. 2



16% Sb, 10% Sn, 0.3% As, 0.0005% S. Magnification 100 X — Etchant, Acetic Acid + H<sub>2</sub>O<sub>2</sub>.

Fig. 2a



16% Sb, 10% Sn, 0.3% As, 0.0044% S. Magnification 100 X — Etchant, Acetic Acid + H<sub>2</sub>O<sub>2</sub>.

Fig. 3



12.5% Sb, 0.75% Sn, 3.0% As, 0.0002% S. Magnification 100 X — Etchant, Acetic Acid + H<sub>2</sub>O<sub>2</sub>.

Fig. 3a



12.5% Sb, 0.75% Sn, 3.0% As, 0.0025% S. Magnification 100 X — Etchant, Acetic Acid + H<sub>2</sub>O<sub>2</sub>.

Inventors

Albert A. Smith, Jr.  
Herbert E. Howe

334

*John F. Keay*  
Attorney

# United States Patent Office

2,695,845

Patented Nov. 30, 1954

1

2,695,845

## ANTIMONIAL LEAD ALLOYS

Albert A. Smith, Jr., Metuchen, and Herbert E. Howe, Plainfield, N. J., assignors to American Smelting and Refining Company, New York, N. Y., a corporation of New Jersey

Application February 15, 1950, Serial No. 144,246

6 Claims. (Cl. 75—166)

This invention relates to antimonial lead alloys and has, as a primary object, the provision of certain of such alloys with improved properties.

It has been found that by incorporating a critical amount of sulphur in certain antimonial lead compositions, that ductility is greatly enhanced and a marked refinement in grain size results with accompanying increase in fatigue strength.

Composition limits of the essential constituents of the various antimonial lead alloys embraced by the invention are: (a) 12–25% Sb, 0.001–0.01% S, balance Pb; (b) alloy (a) with 0.1–20% Sn replacing an equivalent amount of lead; and (c) alloy (b) with 0.1–3.5% as replacing an equivalent amount of lead. Minor impurities and non-essential constituents may be present to the extent that they do not adversely affect or destroy the beneficial effects of the sulphur content.

The marked grain refining effect achieved by the critical sulphur content of the alloys of the invention is best observed by referring to the drawings accompanying this specification in which the several figures show photomicrographs of three pairs of lead-base alloys, each pair of which differ only in sulphur content, with the alloy of the invention in each case being shown in the figure bearing the suffix *a*. The composition of each alloy is shown in each figure except for lead which constitutes the balance of the alloy in all cases.

The superiority of the alloys of the invention with regard to fatigue strength is well illustrated by the following example. Identical samples of an alloy (nominal composition 15% Sb, 1% Sn, 1% As, bal. Pb) were prepared except for the sulphur content which was 0.0002% and 0.0029%, respectively. Test samples of each were poured and the resulting castings tested on a standard R. R. Moore rotating beam fatigue machine with the following results:

| Alloy with— | Load,<br>P. s. i. | Cycles to<br>failure |
|-------------|-------------------|----------------------|
| 0.0002%     | 4,500             | 1,114,400            |
| 0.0029%     | 4,500             | 13,851,700           |

The greatly increased ductility exhibited of the alloys

2

of the invention is readily apparent from the following results of bend tests conducted on alloys (15% Sb, 1% Sn, 1% As, bal. Pb) otherwise identical except for their sulphur contents. This test consists, in general, in bending the specimen ( $\frac{1}{8}$ " x 1" x  $6\frac{1}{2}$ "), which is placed between two rolls, by means of a pin of 0.25" radius moving at constant speed until the first crack appears. The angle of bend is then measured.

| 10 | S content of alloy (percent) | Angle of Bend in<br>Degrees | Average<br>Angle of<br>Bend |
|----|------------------------------|-----------------------------|-----------------------------|
| 15 | 0.0000                       | 9-9-12-10                   | 10°                         |
|    | 0.0012                       | 42-43-41                    | 42°                         |
|    | 0.0032                       | 59-69-77-40-47              | 58°                         |

From a study of the comparative examples shown in the drawings and the results of the tests outlined above, 20 the beneficial effects to be gained by incorporating a proper amount of sulphur in certain antimonial lead alloys are readily apparent. Investigations have shown that the amount of sulphur has to be at least 0.001% and the antimony content of the alloy not less than 12% to 25 initiate the improvement in properties. The limits of the essential constituents in all of the alloy compositions embraced by the invention are as shown earlier in this specification and in the appended claims.

- What is claimed is:
- 30 1. An alloy consisting essentially of 0.001–0.01% sulphur, more than 12% and up to 25% antimony, balance lead.
2. An alloy according to claim 1 in which an equivalent amount of lead is replaced by 0.1–20% tin.
- 35 3. An alloy consisting essentially of 0.001 to 0.01% sulphur, 0.1 to 20% tin, 0.1 to 3.5% arsenic, more than 12% and up to 25% antimony and the balance lead.
4. An alloy consisting essentially of 0.01% sulphur, more than 13% and up to 25% antimony, and the balance lead.
5. An alloy consisting essentially of 0.001% to 0.01% sulphur, more than 13% and up to 25% antimony, and the balance lead.
- 45 6. An alloy as defined in claim 5 which additionally contains small amounts of metal selected from the group consisting of arsenic, tin and mixtures thereof.

## References Cited in the file of this patent

## UNITED STATES PATENTS

| Number    | Name        | Date          |
|-----------|-------------|---------------|
| 1,722,358 | Seljesaeter | July 30, 1929 |

## OTHER REFERENCES

Fink et al., treatise in Trans. Amer. Electrochemical Society, 1941, vol. 79, pages 272, 273 (complete article, pages 269–305).